

M. BICHEROUX.

METHOD OF MANUFACTURING RAW PLATE GLASS.

APPLICATION FILED JUNE 22, 1910.

1,090,904.

Patented Mar. 24, 1914



Witnesses

Katherine Koch  
Daniel Holmgren

Inventor:

Max Bicheroux  
by Briesen & Gumpel  
Attorneys.

# UNITED STATES PATENT OFFICE.

MAX BICHEROUX, OF HERZOGENRATH, GERMANY, ASSIGNOR TO HERZOGENRATHER SPIEGELGLAS- UND SPIEGEL-FABRIK BICHEROUX, LAMBOTTE & CIE., GESELLSCHAFT MIT BESCHRANKTER HAFTUNG, OF HERZOGENRATH, GERMANY.

## METHOD OF MANUFACTURING RAW PLATE-GLASS.

1,090,904.

Specification of Letters Patent. Patented Mar. 24, 1914.

Application filed June 22, 1910. Serial No. 568,260.

To all whom it may concern:

Be it known that I, MAX BICHEROUX, a subject of the King of Belgium, residing at Herzogenrath, Rhineland, Germany, have 5 invented an Improved Method of Manufacturing Raw Plate-Glass, of which the following is a specification.

This invention relates to a novel method of manufacturing raw plate glass, and more 10 particularly to a method of manufacturing thin raw plate glass from a large pour of molten glass.

The essential feature of this invention 15 consists in rolling out said pour into a coherent plate from which a plurality of sheets is consecutively severed in the rear of the roll, and consecutively pushing said severed sheets from the relatively cold surface of the pouring table on to the hot base of an 20 annealing chamber while the rolling out of the molten mass is still proceeding. In this way the lengths of the severed sheets may be so chosen that the temperature differences between the first and last rolled part of each 25 of said sheets are such as to avoid all danger of cracking and the like.

In the accompanying drawing:—Figure 1 is a side view of an apparatus suitable for carrying my invention into effect, Fig. 2 a 30 plan thereof, and Fig. 3 an enlarged cross section through the adjoining sides of a pair of tables.

As shown in Figs. 1 and 2, there are employed a number of small pouring tables  $a$ ,  $a^1$ ,  $a^2$ ,  $a^3$ ,  $a^x$  which are placed behind each other with narrow intervening gaps, so that the tables may expand independently from each other and may be separately cooled if desired. The intervals between the several 40 tables accommodate bars  $b$ ,  $b^1$ ,  $b^2$ ,  $b^3$ ,  $b^x$  which are provided with beveled faces  $c$  resting against the chamfered edges of the tables (Fig. 3). The compound table constructed as described can be lengthened to 45 the extent desired and owing to its subdivisions, possesses such a degree of stability that the production of uniformly heavy raw glass is insured, notwithstanding the heat emanating from the molten glass during continuous manufacture.

The entire dough like contents of the glass pot are poured upon the first table  $a$  in front of the roller  $d$ . By means of the roller,

the molten glass is rolled out into a single plate, extending over all of the tables. The 55 thickness of the plate is determined in known manner, by means of rails  $g$  which are formed either on the roller itself or on the pouring tables.

Corresponding to the progress of the rolling operation, there are severed from the plate, by means of a suitable cutting device  $f$  arranged directly back of roller  $d$ , a plurality of units or individual sections. These sections are divided from each other at or 60 about the abutting points  $b-b^x$ , so that each section possesses the size of a single table  $a-a^x$ . The severed sections are then consecutively pushed from the several tables to the annealing furnace, say in the direction 65  $e$ ,  $e^1$ ,  $e^2$ ,  $e^3$ ,  $e^x$  by applying a pressure to each of said sections on one of its longitudinal edges. This removal takes place while the 70 rolling out of the molten pour is still proceeding.

The size of the several pouring tables as 75 well as the number of such tables used, are dependent upon the particular conditions present.

The invention possesses a number of advantages aside from those alluded to.

Raw plate glass can only be obtained from glass-pots so as to insure the desirable purity of the glass, that is to say invariably a single sheet of glass is obtained from a single 80 glass-pot. As the cost of the manufacture diminishes quite considerably with the size of the glass-pot, it has become a rule to increase such size, in other words to produce sheets of raw glass of an ever increasing 85 size. However the limit has already been attained for the maximum size of from 30 to 35 square meters of the glass plate. It would not be possible further to extend the rolling process, since there would be danger 90 that the part first rolled would crack before the sheet could be moved into the annealing oven. Indeed, as it is, this part frequently cracks in the annealing oven or during the grinding operation. Aside from the above 95 objection, another difficulty is that the glass plate which is moved into the annealing oven, with its last formed end still in a soft state, will under its increasing weight be apt to jam or swell, as is indeed the case. 100 Furthermore, the cooling of the glass plates

with the present sizes is already attended with serious difficulty and inconvenience, which would render the process practically impossible if the size of the plates were to be still further increased. It should also be noted, that for a further extension of the surface of the sheet of glass, no construction of a single piece pouring-table would prove sufficiently stable to insure a uniform thickness of the glass. It has already become a rule to roll on each table at most only 6-8 plates, in order to avoid too great deformations, or to cool the table with water. The new method avoids all these defects and enables pots of any desired capacity to be used for the production of plates of any desired sizes, said plates being during the rolling operation subdivided into a number of units, of which each unit may on account of its small size be treated by itself, so as to overcome the above difficulties. So also, as already stated, the new process permits the formation of raw plate glass of any thinness desired for grinding thin plate glass. The advantage obtained by the employment of large glass-pots is accompanied by a considerable saving in raw material and an essential reduction in the cost of grinding, not to mention the fact that the annealing of the small pieces of crude plate glass produced by the new method in a single rolling operation is cheaper, more even and

less likely to produce cracks than the annealing of a single undivided large plate.

I claim:

1. The method of manufacturing raw plate glass which consists in pouring out a molten mass of glass upon a flat and relatively cool table rolling out a coherent plate from said molten mass, consecutively severing a plurality of sheets from said coherent plate in the rear of the line of rolling, and consecutively removing said severed sheets from the relatively cool surface on to a hot surface while the rolling out of the molten mass is still proceeding.

2. The method of manufacturing raw plate glass which consists in pouring out a molten mass of glass upon a flat and relatively cool table, rolling out a coherent plate therefrom progressively from one end of the flat surface to the other, consecutively severing a plurality of sheets from said coherent plate in the rear of the line of rolling and pushing the severed sheets with a pressure applied on the longitudinal edge of the sheet in a direction transverse to the direction of rolling and over said cool surface on to a hot surface while said rolling of the molten mass is proceeding.

MAX BICHEROUX.

Witnesses:

HENRY QUADFLIEG,  
GUSTAV WEGMANN.